

Oct. 20, 1953

R. C. GUNTHER

2,656,272

STABILIZED AZINE PHOTOGRAPHIC DEVELOPERS CONTAINING  
SODIUM METABORATE AS THE SOLE ALKALI

Filed Nov. 30, 1950

Effect of Developer Storage  
on Maximum Dye Density



Robert C. Gunther  
INVENTOR.

BY *Henry W. Conlon*  
*Edward P. Gilheany*  
ATTORNEYS

## UNITED STATES PATENT OFFICE

2,656,272

## STABILIZED AZINE PHOTOGRAPHIC DEVELOPERS CONTAINING SODIUM METABORATE AS THE SOLE ALKALI

Robert C. Gunther, Galesburg, Ill., assignor to  
General Aniline & Film Corporation, New York,  
N. Y., a corporation of Delaware

Application November 30, 1950, Serial No. 198,396

7 Claims. (Cl. 95—88)

1

The present invention relates to stabilized azine photographic developers, and particularly such developers in which stabilization has been effected by replacing the sodium carbonate generally employed as the alkali by sodium metaborate.

United States Letters Patent 2,486,440 granted November 1, 1949, to Schmidt and Tulagin, and my United States Letters Patent 2,570,116, issued October 2, 1951, describe azine color developers in which the essential components are a 2,4-diamino aniline and an alkali, specifically sodium carbonate.

In order to be commercially feasible, a developer for the production of azine dye images in photographic elements should possess the following general characteristics:

- (a) Good storage stability;
- (b) The ability to produce maximum dye density in minimum time;
- (c) The ability to produce a minimum of proximity development; and
- (d) Satisfactory development characteristics, such as rate of development, slow rate of exhaustion, and the like.

The effective developing agent in the azine developers described in the foregoing patent and application, being a diamino aniline derivative, is very susceptible to aerial oxidation, and this factor has long presented a serious stability problem in the preparation and use of azine color developer solutions.

Although the storage stability requirements for an azine color developer cannot be too well defined, nevertheless it is felt that such a developer should be stable, with moderate use for at least a week to ten days, without change in its color development properties.

Efforts have been made to improve the storage stability of the azine developers by including components specifically designed to preserve the developers. To this end there have been used dextrose, hydroxylamine, p-hydroxyphenylglycine and Rongalite, among others. While certain of these compounds, specifically hydroxylamine, have a definite stabilizing action, each of the compounds tested had a deleterious effect on the development properties of the color developers. Thus, dextrose, p-hydroxyphenylglycine and Rongalite decrease the development potential. On the other hand, the hydroxylamine causes a serious loss in color rendition by increasing proximity development.

In view of the results involving the employment of additives, to improve azine developer stability, it was realized that some other means

5 would have to be found if developers of satisfactory storage stability were to be produced. As a result of this conclusion, I discovered, rather surprisingly, that developers of satisfactory stability could be obtained by replacing the sodium carbonate used to supply alkalinity to the known azine developers by sodium metaborate. By this substitution of the sodium metaborate for sodium carbonate, it was found that the developers with the sodium metaborate were many times more stable than the developers containing sodium carbonate.

10 Color developers of the 2,4-diaminoaniline class, containing sodium metaborate, as the alkali and as a stabilizer for the developer, constitute the purposes and objects of the present invention.

15 The quantity of the sodium metaborate which I found to be effective ranges from about 30 to 50 parts per liter of developer. With this amount of sodium metaborate, the stability of the developer composition is two to three times as great as the stability of a corresponding developer containing sodium carbonate as the alkali. Such improved stability manifests itself not only by a 20 slower darkening rate of the solution itself, but also by an improved color brilliance and maximum dye density.

25 It is evident from what has been said, that the essential components of my developer are a 2,4-diaminoaniline as the effective reducing agent and sodium metaborate as the alkali. As the 30 2,4-diaminoaniline, I may use any one of those which are described in the aforesaid United States Letters Patent 2,486,440, or in my aforesaid U. S. Patent 2,570,116.

35 Examples of such 2,4-diaminoanilines are: 4-( $\beta$ -hydroxyethylamino)-6-phenylaminometanilic acid; 4,6-di( $\beta$ -hydroxyethylamino)-metanilic acid; 4-( $\beta$ -hydroxyethylamino)-6-(4'-carboxy-methoxyphenylamino)-metanilic acid; 4-(o-methoxyphenylamino)-6-(p-methoxyphenylamino)-metanilic acid, and the like.

40 In addition to the 2,4-diaminoaniline and the alkali, the developer should contain the usual adjuncts, such as an alkali metal sulfite, i. e. sodium sulfite, potassium sulfite and the like, an alkali metal bromide such as potassium bromide and the like, and a coupling aid such as pyridine, benzylamine and the like.

45 In my U. S. Patent 2,594,917 I discussed the phenomenon known as "proximity development" and suggest that this may be suppressed by the utilization of a phenol. U. S. Patent 2,596,926 suggests the utilization of amino pyridines for the same purpose. It is, therefore, advisable to 50

## 3

include either a phenol or an amino pyridine in the developer, to reduce proximity development. Sodium sulfate, which is also found to have a similar effect, may also be employed.

In my U. S. Patent 2,623,823 I discuss energizers for 2,4-diaminoaniline developers, which are the reaction product of such a developer, with an aldehyde or pyruvic acid, or a derivative thereof. Such compounds also aid in giving a developer of optimum characteristics.

The proportions of the various components in the developer may vary, but I have found that the developers constituted as noted below are very effective:

|                                                                                                             | Parts | 15  | 10   | 10 |
|-------------------------------------------------------------------------------------------------------------|-------|-----|------|----|
| A 2,4-diaminoaniline                                                                                        | 4 to  | 8   |      |    |
| Sodium metaborate anhydrous                                                                                 | 20 to | 60  |      |    |
| An alkali metal sulfite                                                                                     | 20 to | 60  |      |    |
| An alkali metal bromide                                                                                     | 1 to  | 5   |      |    |
| An amino pyridine                                                                                           | 1 to  | 20  | 20   |    |
| The reaction product of a 2,4-diamino aniline with an aldehyde or with pyruvic acid or a derivative thereof | 2 to  | 4   |      |    |
| A phenol                                                                                                    | 0 to  | 10  |      |    |
| Sodium sulfate                                                                                              | 50 to | 150 | 25   |    |
| Ascorbic acid                                                                                               | 0 to  | 3   |      |    |
| Water to make                                                                                               |       |     | 1000 |    |

It is evident that the ascorbic acid is not necessarily present in the developer. It has been found, however, that while ascorbic acid in a developer containing sodium carbonate as the alkali is not a satisfactory stabilizer, nevertheless when used in a developer containing sodium metaborate as the alkali, it increases the stability beyond that afforded by the sodium metaborate alone. Consequently, for best results it is preferred to include ascorbic acid in the composition.

The following examples will serve to illustrate developer compositions for the azine synthesis, which I have found to have a storage stability much greater than that possessed by known developers containing sodium carbonate as the alkali.

## EXAMPLE 1

|                                                                                                                       | Grams |
|-----------------------------------------------------------------------------------------------------------------------|-------|
| 4-( $\beta$ -hydroxyethylamino) - 6 - phenylamino metanilic acid                                                      | 5     |
| Sodium metaborate (86%)                                                                                               | 30    |
| Sodium sulfite                                                                                                        | 60    |
| Potassium bromide                                                                                                     | 1     |
| 2-amino pyridine                                                                                                      | 16    |
| The reaction product of pyruvic acid with 4-( $\beta$ - hydroxyethylamino) -6-phenylamino metanilic acid <sup>1</sup> | 3     |
| Sodium sulfate                                                                                                        | 100   |
| Water to make 1000 cc.                                                                                                |       |

<sup>1</sup>(Hereinafter referred to as the Energizer)

## EXAMPLE 2

The composition is the same as Example 1, excepting that it includes 1 gram of ascorbic acid.

## EXAMPLE 3

|                                                                  | Grams |
|------------------------------------------------------------------|-------|
| 4-( $\beta$ -hydroxyethylamino) - 6 - phenylamino metanilic acid | 5     |
| Sodium metaborate (86%)                                          | 50    |
| Sodium sulfite                                                   | 40    |
| Potassium bromide                                                | 1     |
| 2-amino pyridine                                                 | 16    |
| Energizer                                                        | 3     |
| Sodium sulfate                                                   | 100   |
| Water to make 1000 cc.                                           |       |

## 4

## EXAMPLE 4

The composition is the same as that of Example 3, excepting that it includes 1 gram of ascorbic acid.

In order to establish the improvement wrought by the utilization of sodium metaborate, in lieu of sodium carbonate, in azine developers, I compounded the following developers for comparison with those of the examples.

## A

|                                                                  | Grams |
|------------------------------------------------------------------|-------|
| 4-( $\beta$ -hydroxyethylamino) - 6 - phenylamino metanilic acid | 5     |
| Sodium carbonate monohydrate                                     | 40    |
| Sodium sulfite                                                   | 60    |
| Potassium bromide                                                | 5     |
| Pyridine                                                         | 16    |
| Benzylamine                                                      | 1     |
| Phenol (in 100 cc. of 10% trisodium phosphate)                   | 10    |
| Energizer                                                        | 2.5   |
| Water to make 1000 cc.                                           |       |

## B

|                                                                  | Grams |
|------------------------------------------------------------------|-------|
| 4-( $\beta$ -hydroxyethylamino) - 6 - phenylamino metanilic acid | 5     |
| Sodium carbonate monohydrate                                     | 40    |
| Sodium sulfite                                                   | 60    |
| Potassium bromide                                                | 5     |
| 2-amino pyridine                                                 | 16    |
| Phenol (in 100 cc. of 10% trisodium phosphate)                   | 10    |
| Energizer                                                        | 2.5   |
| Water to make 1000 cc.                                           |       |

Reference is here made to the fact that the proportioning of the ingredients in these two developers is designed to give optimum results with the components employed.

There are three methods known for comparing the stability of the developers containing sodium carbonate on the one hand, and those containing metaborate on the other hand, and these are as follows:

(1) Comparison of color of the stored developer compositions;

(2) Comparison of maximum density on development of the same sensitometric, photographic strips at various periods of developer storage time; and

(3) Comparison of relative color brilliance of the spectrograms photographically developed in the aged developer solutions.

The first comparison is a visual one, and hence requires no detailed discussion.

In making the other two comparisons, I utilized as the sensitometric strips, azine multi-layer film prepared as follows:

On a film base was cast a red sensitive silver halide emulsion layer containing as a cyan color former, one of the fast to diffusion aryl J acids described in U. S. Patent 2,591,642. On the red sensitive layer was cast a green sensitive silver halide emulsion layer containing as the magenta color former, one of the fast to diffusion 8-hydroxy quinolines disclosed in United States Letters Patent 2,524,725 granted on October 3, 1950, to Robert F. Coles. Over the green sensitive layer was cast a blue sensitive silver halide emulsion layer containing as the yellow color former, one of the benzimidazole derivatives, fast to diffusion, described in United States Letters Patent 2,500,487 granted on March 14, 1950 to Winfred C. Craig.

Each film prepared as above was utilized by exposing it to a spectrum, developing it in black and white, re-exposing and developing it in the test solution; i. e. the solutions containing sodium carbonate characterized as A and B above, and the solutions of the examples.

The specific procedure followed in utilizing such color developers involves the following steps:

(1) Spectrograms were made using fresh developer solution;

(2) The developers were stored twelve days with periodic use, 400 square inches of azine color film being developed per liter of solution;

(3) Spectrograms were made using the old developers, i. e. after twelve days' storage;

(4) Color density measurements were made on the spectrograms from the fresh developer solutions ("before"), and from the old developer solutions ("after").

The results of these tests are indicated in the table below, it being pointed out that developer 1 in said table is solution A above, containing sodium carbonate, 2 is solution B above containing sodium carbonate, and 3 to 6 inclusive corresponding to Examples 1 to 4, respectively.

TABLE

| Developer Number | D max. |       | dr 640 $\mu$ |       | Relative Color Brilliance |       | Relative Developer Stability<br>$\frac{D \text{ max. (a)}}{dr 640\mu \text{ (a)}} \times 100$ | Color of Solution After Storage |  |  |
|------------------|--------|-------|--------------|-------|---------------------------|-------|-----------------------------------------------------------------------------------------------|---------------------------------|--|--|
|                  | Before |       | After        |       | D max.<br>dr 640 $\mu$    |       |                                                                                               |                                 |  |  |
|                  | Before | After | Before       | After | Before                    | After |                                                                                               |                                 |  |  |
| 1.....           | 2.35   | 1.77  | 0.29         | 0.55  | 8.1                       | 3.2   | 39.5                                                                                          | Deep red.                       |  |  |
| 2.....           | 2.02   | 1.70  | 0.25         | 0.50  | 8.1                       | 3.4   | 42.0                                                                                          | Do.                             |  |  |
| 3.....           | 2.26   | 2.08  | 0.19         | 0.33  | 11.9                      | 6.3   | 52.9                                                                                          | Orange-yellow.                  |  |  |
| 4.....           | 2.10   | 1.93  | 0.18         | 0.21  | 11.7                      | 9.2   | 78.6                                                                                          | Yellow.                         |  |  |
| 5.....           | 2.38   | 2.29  | 0.19         | 0.29  | 12.5                      | 7.9   | 63.2                                                                                          | Orange-yellow.                  |  |  |
| 6.....           | 2.30   | 2.16  | 0.18         | 0.21  | 12.8                      | 10.3  | 80.5                                                                                          | Yellow.                         |  |  |

## NOTES:

(1) In column 5 of the table, (a) means "after" and (b) in the same column refers to "before."

(2) dr in the table refers to the cyan density through the red filter at 640 $\mu$ .

(3) The color brilliance of any one spectrum was taken as the ratio of the maximum neutral density to the cyan density through a red filter at 640 $\mu$ .

(4) The maximum density was determined by use of the commercial "Ansco-Sweet" black and white densitometer.

It will be observed that this table gives not only the color change of the solutions on storage, but also gives the maximum densities and relative color brilliance of the fresh solutions and of the solutions upon aging. It will also be observed that the developers containing sodium metaborate are far and away more stable than those containing sodium carbonate.

Attention is also directed to the attached drawing which shows graphically the effect of development storage on maximum dye densities of the six solutions of the table.

It will be appreciated that solution 2 is very similar to solution 5, excepting that a small amount of phenol is present in solution 2. By comparing curves 2 and 5 of the drawing, after twelve days' storage, it will be found that the metaborate containing developer showed a loss of D<sub>max</sub> of .1 of a unit, whereas the carbonate containing developer over the same storage time showed a loss in D<sub>max</sub> of .3 of a unit.

Curve 3 indicates that by storage of the developer thereof for twelve days, the loss in D<sub>max</sub> is only .15 of a unit. If an attempt be made to alter the formula of developer composition of curve 5 by substituting half of the sodium metaborate by sodium carbonate, a developer composition results which possesses storage properties much inferior to those of the developer of curve 5.

Reference has previously been made to the fact that ascorbic acid, when present in a small amount in a developer containing metaborate, further promotes the stability of the developer. This fact is emphasized by this additional test: Developers 1 to 5 of the table were allowed to stand in capped amber bottles for two months after the tests described in the table were completed. At the end of this time, all of the developers, except 4, were a very dark red color. Developer 4, the only one containing ascorbic acid, was still a light orange-yellow color. Upon development of step wedges and spectrograms with the 5 solutions, No. 4 produced images of excellent brilliance and very clear whites, whereas none of the other developers produced any dye image whatsoever. It will thus be seen that a small amount of ascorbic acid operates to greatly promote the stabilizing effect of the sodium metaborate.

It has been proposed in the past to utilize sodium metaborate in fine grain black and white developers, and, in fact, this product is commercially offered for use in this relationship. There is no suggestion, however, in any prior art which

would lead one to believe that sodium metaborate has a very marked stabilizing effect on azine developers when used as the alkali thereof.

Various modifications of the invention will be apparent to persons skilled in the art, and I, therefore, do not intend to be limited in the patent granted except as required by the appended claims.

I claim:

1. A storage stable developer solution for the production of azine dyestuff images containing a 2,4-diaminoaniline and sodium metaborate as the only alkali for the developer.
2. The composition as defined in claim 1, wherein the 2,4-diaminoaniline is 4-( $\beta$ -hydroxyethylamino)-6-phenylamino metanilic acid.
3. The composition as defined in claim 1, containing in addition, sodium sulfite and potassium bromide.
4. The composition as defined in claim 1, wherein the sodium metaborate is present in a concentration of from 30 to 50 grams per liter of developer solution.
5. A storage stable developer solution for the preparation of azine dye images containing 4-( $\beta$ -hydroxyethylamino)-6-phenylamino metanilic acid, sodium metaborate as the only alkali for the developer and a small amount of ascorbic acid.
6. A storage stable developer solution for the

preparation of azine dye images of the following composition:

|                         | Parts    |
|-------------------------|----------|
| A 2,4-diaminoaniline    | 4 to 8   |
| Sodium metaborate       | 20 to 60 |
| An alkali metal sulfite | 20 to 60 |
| An alkali metal bromide | 1 to 5   |
| An amino pyridine       | 1 to 20  |

The reaction product of a 2,4-diaminoaniline with a compound selected from the class consisting of those of the following formulae: R<sub>4</sub>—CHO and R<sub>5</sub>—COCOOH

|                                                                                     | Parts   |
|-------------------------------------------------------------------------------------|---------|
| R <sub>4</sub> being selected from the class consisting of hydrogen and lower alkyl | 15      |
| and R <sub>5</sub> being lower alkyl                                                | 2 to 4  |
| A phenol                                                                            | 0 to 10 |

|                | Parts     |
|----------------|-----------|
| Sodium sulfate | 50 to 150 |
| Ascorbic acid  | 0 to 3    |
| Water to make  | 1000      |

7. The composition as defined in claim 1 containing up to 3 parts of ascorbic acid.

ROBERT C. GUNTHER.

References Cited in the file of this patent

UNITED STATES PATENTS

| Number    | Name          | Date           |
|-----------|---------------|----------------|
| 2,018,657 | Bennett       | Oct. 29, 1935  |
| 2,384,663 | Weissberger   | Sept. 11, 1945 |
| 2,401,713 | Vittum et al. | Jan. 4, 1946   |
| 2,414,491 | Tulagin       | Jan. 21, 1947  |
| 2,527,379 | Schmidt       | Oct. 24, 1950  |